

May 13, 1941.

A. S. BELL ET AL

2,241,442

PROCESS OF PRODUCING COMPOSITE YARNS

Filed April 1, 1939

FIG. 1



FIG. 2



FIG. 3



FIG. 4



Inventors:

A. S. Bell

J. R. Wyde

G. Kelly, ad b. Bergmann

Attorneys

## UNITED STATES PATENT OFFICE

2,241,442

PROCESS OF PRODUCING COMPOSITE  
YARNS

Angus Smith Bell and Joseph Rowland Wylde,  
Spondon, near Derby, England, assignors to  
Celanese Corporation of America, a corpora-  
tion of Delaware

Application April 1, 1939, Serial No. 265,485  
In Great Britain June 7, 1938

12 Claims. (Cl. 57—157)

This invention relates to improvements in composite yarns and in fabrics and other materials containing such yarns.

In British Patent No. 482,425, processes are described wherein composite yarns resembling wool yarns are produced by associating together, preferably by a doubling twist, one or more yarns of crinkled cellulose acetate filaments with one or more high twist yarns, the said yarn or yarns of crinkled cellulose acetate filaments being present in the composite yarn produced in substantially greater proportion than the said high twist yarn or yarns and having in the composite yarn produced at most only a low degree of twist, and the said high twist yarn or yarns having in the composite yarn produced a degree of twist such that they possess the ability to shrink on treatment with hot aqueous liquors. Again, in British Patent No. 482,376, processes are described wherein composite yarns resembling wool yarns are produced by associating together, preferably by a doubling twist, one or more yarns of crinkled artificial filaments, which preferably have a basis of a material other than cellulose acetate, with one or more highly twisted yarns, said yarn or yarns of crinkled artificial filaments having in the composite yarn at most only a low degree of twist and the said yarns of high twist being in the composite yarn so highly twisted that they possess the ability to shrink on treatment with hot aqueous liquors. Also, in British Patent No. 482,376, processes are described wherein composite yarns resembling wool yarns are obtained by associating one or more yarns of crinkled artificial filaments with one or more yarns capable of being shrunk relatively to the said yarn or yarns of crinkled artificial filaments and thereafter shrinking the said shrinkable yarns, the said yarn or yarns of crinkled artificial filaments having in the composite yarn at most only a low degree of twist, and the said shrinkable yarn or yarns having in the composite yarn a degree of twist less than crêpe twist.

It has now been discovered that particularly valuable composite yarns may be produced by doubling two or more yarns of uncrinkled filaments with one or more yarns of crinkled filaments, the yarn or yarns of crinkled filaments being fed to the doubling device at a greater speed than the yarns of uncrinkled filaments, and the yarns of uncrinkled filaments being fed to the doubling device in at least two different directions. In this way composite yarns may be obtained which have excellent voluminosity and in which the individual yarns of crinkled filaments

are very well secured in position so that such yarns have very little tendency to slip along the yarns of uncrinkled filaments and thus form slubs.

5 The invention is of particular importance in connection with the production of composite yarns containing yarns of crinkled cellulose acetate filaments. Crinkled filaments of cellulose acetate are obtained by subjecting bundles or 10 yarns of cellulose acetate filaments, especially such as comprise filaments of flat or nearly flat cross-section, to the action of hot or boiling water, or preferably hot or boiling dilute soap solutions. The flat type of filament is preferably produced by spinning a cellulose acetate solution in a normal way into an evaporative atmosphere but using a concentration of cellulose acetate in the acetone or other volatile solvent lower than is customarily used to produce the bulbous type 15 of filament. However, the flat type of filament may also be produced by spinning the cellulose acetate solution into an evaporative atmosphere which contains a high concentration of solvent for cellulose acetate near the spinning jets. Alternatively, or in addition, the spinning solution 20 may contain paradichlorbenzene or other plasticising agent as described in British Patent No. 459,781. Other things being equal, a higher degree of crinkling, and therefore of voluminosity, is obtained with the higher filament deniers. The crinkling of the cellulose acetate filaments may be effected, for example, by treating such filaments, e. g. in the form of hanks of yarn, with hot aqueous liquors, and especially with hot dilute 25 soap solutions, without tension so as to develop the crinkle in the filaments. The crinkle developed by the above processes is irregular in character.

Again, crinkle is imparted to cellulose acetate 30 filaments by processes such as those described in U. S. Patents Nos. 2,089,198, 2,089,199 and 2,111,211. These processes consist, broadly, in imparting a twist to the yarns, setting the twist in the yarns, e. g. by the action of steam, and thereafter untwisting the yarns. Preferably the operation is effected with a false twisting device. Such processes impart a spiral crinkle to the filaments. If desired, the crinkling of the filaments may be accomplished by a combination of the two methods described above, e. g. a yarn or bundle of flat filaments of cellulose acetate may be subjected to one of the processes of U. S. Patents Nos. 2,089,198, 2,089,199 and 2,111,211 and either before or after such treatment, subjected 35 to the action of hot aqueous liquors.

The yarns of crinkled filaments may have a basis of materials other than cellulose acetate. Thus, they may comprise filaments of any other organic derivative of cellulose, regenerated cellulose, e. g. viscose, cuprammonium and nitro-cellulose artificial silks, or partially or completely saponified cellulose acetate or other cellulose ester artificial silk. Or again, the yarns of crinkled filaments may have a basis of cellulosic material but have been subjected to a process of surface esterification or etherification, or may have a basis of an organic derivative of cellulose and have been subjected to a process of esterification, e. g. as described in U. S. Patents Nos. 2,159,011 and 2,159,012 and British Patent No. 448,817. Crinkled artificial filaments contained in the yarns may have been subjected to a stretching process or a shrinking process prior to their association with the yarns of uncrinkled filaments in accordance with this invention. Any stretching operation should, of course, be carried out prior to imparting crinkle to the filaments.

The crinkled filaments in the yarns may be continuous or may be discontinuous, provided that the length of the staple in the product is not so short as to necessitate a relatively high degree of twist to produce a coherent product. A staple length of 5-8 or 10 inches or more may be used but preferably the staple is as long as possible, e. g. of the order of 18 inches.

The yarns of uncrinkled filaments may be made of any suitable material, e. g. the materials specified above for the yarns of crinkled filaments. It is especially advantageous to employ yarns of high tenacity, e. g. 2.5 or more grams per denier, as the yarns of uncrinkled filaments, for example cellulose acetate yarns which have been stretched considerably so as to impart to them a tenacity of about 3.5 gms. per denier or more, or the products obtained by partial or complete saponification of such yarns. By employing yarns of considerable strength as the yarns of uncrinkled filaments it is possible to double with them relatively large quantities of the yarns of crinkled filaments and thus increase the total voluminosity of the product while conserving the necessary strength for the product considered as a whole.

Novel effects may be obtained according to this invention by employing in the construction of the composite yarns, individual yarns some of which are coloured and the remainder uncoloured or which are coloured in different colours.

As stated above it is essential according to the present invention that the yarn or yarns of crinkled filaments should be fed to the doubling device at a higher speed than the yarns of uncrinkled filaments. Speeds of 50% or more, and especially from 100 to 300%, faster than that of the yarns of uncrinkled filaments are suitable. In this way the yarn or yarns of crinkled filaments appear in the composite products as if they were more or less spiralled round the yarns of uncrinkled filaments, with the result that the latter may be more or less embedded in the composite product.

It is further essential according to the present invention that the yarns of uncrinkled filaments (of which at least two must be employed) should be fed to the doubling device in different directions. It is not essential, however, that the packages from which such yarns are withdrawn should be widely spaced apart, and it is suffi-

cient to lead two such yarns to the doubling device together and to cause them to pass on opposite sides of an obstruction, such as a smooth bar, just before they reach the point where the twist commences to be inserted, so that they converge on this point from different directions. Thus, using a downward twisting device provided above the twisting spindle with a guide through which the yarns to be twisted are led, a rigid bar may be mounted just above such guide and the yarns of uncrinkled filaments caused to pass on opposite sides of such bar so that they converge on the guide at an angle to one another.

If desired there may be employed as the yarns of uncrinkled filaments, yarns which are capable of being shrunk relatively to the yarns of crinkled filaments. Thus, there may be employed as yarns of uncrinkled filaments the high twist crêpe yarns and other shrinkable yarns described in British Patents Nos. 482,425 and 482,376, referred to above. If such shrinkable yarns are employed they may, if desired, be shrunk in the composite yarns, e. g. before incorporating the composite yarns in a fabric, the shrinking being effected by any of the methods described in the said applications.

By employing according to the invention high twist crêpe yarns or other yarns of high extensibility as the yarns of uncrinkled filaments, products may be obtained which not only resemble chenille yarns in appearance but have the additional advantage of a much greater extensibility than ordinary cotton/wool chenille yarns.

The doubling twist used to double together the 35 yarns of uncrinkled filaments and the yarn or yarns of crinkled filaments is preferably only low and should not be so high as to reduce substantially the voluminosity. As a result of the doubling operation the yarns of uncrinkled filaments either receive twist or have some twist removed from them, depending on the relative directions of the twist in such yarns and of the doubling twist. For this reason the twist in the yarns of uncrinkled filaments before the doubling operation should be either in excess of or short of that desired for them in the ultimate product. Where the yarns of uncrinkled filaments are high twist crêpe yarns it is preferable to insert the doubling twist in the same direction as the original twist in such yarns so that at no stage have such yarns a twist higher than that desired for them in the product. By this means the strength of the yarns of uncrinkled filaments is conserved. For example where an ultimate twist of 55 turns 50 per inch in the yarns of uncrinkled filaments of the composite product is desired it is better to insert a twist of 50 turns per inch and then increase this to 55 by a doubling twist of 5 turns per inch in the same direction than to start with an original twist of 60 turns per inch and to decrease this to 55 by a doubling twist of 5 turns per inch in the reverse direction.

As indicated above it is essential that at least two yarns of uncrinkled filaments are employed. More than two of such yarns may, however, be employed if desired, e. g. to make a heavier product. Again more than one yarn of crinkled filaments may be employed. The composite yarns obtained may themselves be doubled together to form composite yarns of greater denier. They may also be doubled with yarns of other types, e. g. normal yarns or high twist crêpe yarns, for producing other effect yarns.

Examples illustrating the production of composite yarns according to the invention will now

be described with reference to Figs. 1-4 of the accompanying diagrammatic drawing.

In the drawing—

A is a 75 denier low twist yarn of normal cellulose acetate filaments;

B is a 200 denier low twist yarn of crinkled cellulose acetate filaments;

C is a 140 denier low twist yarn of normal cellulose acetate filaments;

D is a 150 denier low twist yarn of crinkled cellulose acetate filaments, dyed to a suitable colour;

E is a 100 denier low twist yarn of crinkled cellulose acetate filaments;

F is a 55 denier high tenacity low twist yarn of regenerated cellulose filaments;

G is a 55 denier high tenacity high twist (48 t. p. i. "Z" twist) yarn of regenerated cellulose filaments; and

H is a 170 denier low twist yarn of crinkled cellulose acetate filaments.

Yarns F and G may for example have been produced by completely saponifying a cellulose acetate yarn which has been stretched to 500 or 1000% of its original length in wet steam as described in U. S. Patent No. 2,142,721.

Referring to Fig. 1, two ends of the yarn A are delivered from one feed roller over a tension bar to a doubling device. Just before reaching the doubling device these ends are caused to pass on opposite sides of a bar so that they converge on the doubling device in different directions. One end of the yarn B is delivered from a separate feed roller to the doubling device, the rate of feed being adjusted so that for every 100 units of length of each of the yarns A delivered to the doubling device 300 units of length of the yarn B are delivered. A doubling twist of 36 t. p. i. ("Z" twist) is inserted by the doubling device. Two doubled yarns thus obtained are then doubled together with a doubling twist of 12 t. p. i. ("S" twist).

In Fig. 2, two ends of the yarn C are led to the doubling device in the manner described above with reference to the yarns A, and three ends of yarn D are fed from a separate feed roller to the doubling device, the rate of feed being adjusted so that for every 100 units of length of each of the yarns C 300 units of length of yarn D are delivered. A doubling twist of 29 t. p. i. ("Z" twist) is inserted. Two doubled yarns thus obtained are then doubled together with a doubling twist of 12 t. p. i. ("S" twist).

Fig. 3 illustrates a process in which two ends of yarn A are led to the doubling device as above and one end of each of yarns D and E are fed to the device at a rate of feed such that for every 100 units of length of each yarn A 300 units of length of yarn D and of yarn E are delivered. A doubling twist of 36 t. p. i. ("Z" twist) is inserted and two doubled yarns thus obtained are then doubled together with a doubling twist of 10 t. p. i. ("S" twist).

In Fig. 4 an end of yarn F and an end of yarn G are led to the doubling device in the manner described above with regard to yarns A and an end of yarn H is fed from a separate feed roller at a rate of feed such that for every 100 units of length of yarn F and of yarn G 300 units of length of yarn H are delivered. A doubling twist of 34 t. p. i. ("Z" twist) is inserted and two yarns so formed are then doubled together with a doubling twist of 12 t. p. i. ("S" twist).

The composite yarns produced according to the above examples closely resemble chenille yarns. It will be understood that in any of these

examples other yarns of crinkled filaments and other yarns of uncrinkled filaments may be substituted for those specified and that any of the yarns mentioned may, if desired, be coloured. Further, the three ends of yarn D referred to in Fig. 2 may be similarly coloured or they may be coloured differently from each other.

Having described our invention what we desire to secure by Letters Patent is:

1. Process for the production of composite yarns, which comprises doubling two or more yarns of uncrinkled filaments with one or more yarns of crinkled filaments, the yarns of crinkled filaments being fed to the doubling device at a greater speed than the yarns of uncrinkled filaments, at least two of the yarns of uncrinkled filaments being fed to the doubling device at an angle to each other, so that the yarns of crinkled filaments are caught at intervals between the yarns of uncrinkled filaments.

2. Process according to claim 1, wherein at least one of the component yarns is colored.

3. Process for the production of composite yarns, which comprises doubling two or more yarns of uncrinkled filaments with one or more yarns of crinkled filaments having a basis of an organic derivative of cellulose, the yarns of crinkled filaments being fed to the doubling device at a greater speed than the yarns of uncrinkled filaments, at least two of the yarns of uncrinkled filaments being fed to the doubling device at an angle to each other, so that the yarns of crinkled filaments are caught at intervals between the yarns of uncrinkled filaments.

4. Process for the production of composite yarns which comprises doubling two or more yarns of uncrinkled filaments with one or more yarns of crinkled filaments, the yarns of crinkled filaments being delivered to the doubling device at a speed at least 50% faster than the speed of delivery of the yarns of uncrinkled filaments, at least two of the yarns of uncrinkled filaments being fed to the doubling device at an angle to each other, so that the yarns of crinkled filaments are caught at intervals between the yarns of uncrinkled filaments.

5. Process for the production of composite yarns which comprises doubling two or more yarns of uncrinkled filaments with one or more yarns of crinkled filaments having a basis of an organic derivative of cellulose, the yarns of crinkled filaments being delivered to the doubling device at a speed at least 50% faster than the speed of delivery of the yarns of uncrinkled filaments, at least two of the yarns of uncrinkled filaments being fed to the doubling device at an angle to each other; so that the yarns of crinkled filaments are caught at intervals between the yarns of uncrinkled filaments.

6. Process for the production of composite yarns which comprises doubling two or more yarns of uncrinkled filaments with one or more yarns of crinkled filaments, the yarns of crinkled filaments being delivered to the doubling device at a speed 100-300% faster than the speed of delivery of the yarns of uncrinkled filaments, at least two of the yarns of uncrinkled filaments being fed to the doubling device at an angle to each other, so that the yarns of crinkled filaments are caught at intervals between the yarns of uncrinkled filaments.

7. Process for the production of composite yarns which comprises doubling two or more yarns of uncrinkled filaments with one or more

yarns of crinkled filaments relatively to which said yarns of uncrinkled filaments are capable of being shrunk, the yarns of crinkled filaments being fed to the doubling device at a greater speed than the yarns of uncrinkled filaments, at least two of the yarns of uncrinkled filaments being fed to the doubling device at an angle to each other, so that the yarns of crinkled filaments are caught at intervals between the yarns of uncrinkled filaments.

8. Process for the production of composite yarns which comprises doubling two or more high twist crepe yarns of uncrinkled filaments with one or more yarns of crinkled filaments relatively to which said yarns of uncrinkled filaments are capable of being shrunk, the yarns of crinkled filaments being fed to the doubling device at a greater speed than the yarns of uncrinkled filaments, at least two of the yarns of uncrinkled filaments being fed to the doubling device at an angle to each other, so that the yarns of crinkled filaments are caught at intervals between the yarns of uncrinkled filaments.

9. Process for the production of composite yarns which comprises doubling two or more high twist crepe yarns of uncrinkled filaments with one or more yarns of crinkled filaments, the yarns of crinkled filaments being delivered to the doubling device at a speed 100-300% faster than the speed of delivery of the yarns of uncrinkled filaments, at least two of the yarns of uncrinkled filaments being fed to the doubling device at an angle to each other, so that the yarns of crinkled filaments are caught at intervals between the yarns of uncrinkled filaments.

10. Process for the production of composite yarns which comprises doubling two or more yarns of uncrinkled high tenacity filaments hav-

ing a basis of an organic derivative of cellulose with one or more yarns of crinkled filaments, the yarns of crinkled filaments being fed to the doubling device at a greater speed than the yarns of uncrinkled filaments, at least two of the yarns of uncrinkled filaments being fed to the doubling device at an angle to each other, so that the yarns of crinkled filaments are caught at intervals between the yarns of uncrinkled filaments.

11. Process for the production of composite yarns which comprises doubling two or more yarns of uncrinkled high tenacity filaments having a basis of an organic derivative of cellulose with one or more yarns of crinkled filaments, the yarns of crinkled filaments being delivered to the doubling device at a speed at least 50% faster than the speed of delivery of the yarns of uncrinkled filaments, at least two of the yarns of uncrinkled filaments being fed to the doubling device at an angle to each other, so that the yarns of crinkled filaments are caught at intervals between the yarns of uncrinkled filaments.

12. Process for the production of composite yarns which comprises doubling two or more yarns of uncrinkled filaments with one or more yarns of crinkled filaments, at least one of the component yarns having a basis of cellulose acetate, the yarns of crinkled filaments being fed to the doubling device at a greater speed than the yarns of uncrinkled filaments, at least two of the yarns of uncrinkled filaments being fed to the doubling device at an angle to each other, so that the yarns of crinkled filaments are caught at intervals between the yarns of uncrinkled filaments.

ANGUS SMITH BELL.  
JOSEPH ROWLAND WYLDE.